

# United States Patent Office

3,386,827  
Patented June 4, 1968

1

3,386,827

**THERMO-DEVELOPABLE LIGHT-SENSITIVE DIAZO COMPOSITIONS AND ELEMENTS**  
Claude M. Aebi, Endicott, and Harry F. Herbrandon, Schenectady, N.Y., assignors to International Business Machines Corporation, New York, N.Y., a corporation of New York  
No Drawing. Filed Aug. 17, 1964, Ser. No. 390,240  
4 Claims. (Cl. 96—91)

The present invention relates to light-sensitive diazo-type compositions which are developable by heat. The present invention also relates to light-sensitive diazotype elements, such as films or copying papers which comprise self-supporting films of the compositions or a suitable substrate coated on at least part of one surface with the present compositions.

Thermo-developable, light-sensitive diazotype compositions and elements are well known and are of various types. Some contain acid stabilizers which are decomposed by heat to alter the pH of the system. Others contain compounds which decompose upon heating to form a base, thus also altering the pH of the system to a level at which the color-forming reaction may proceed between the light-sensitive salt and a coupling component present in the composition. Still other thermo-developable systems contain compounds which decompose upon heating to produce coupling components in situ for reaction with the light-sensitive diazonium salt.

The present invention relates to new light-sensitive diazotype compositions and elements comprising compounds of a class which may serve as pH modifiers and/or coupler generators. The compounds present in the composition of this invention are any of those having the following formula:



where  $R_1$  and  $R_2$  may be any radical selected from the group consisting of



and where  $R_3$ ,  $R_4$ ,  $R_5$ ,  $R_6$  and  $R_7$  may be any radical selected from the group consisting of —H, a substituted or unsubstituted alkyl group having from 1 to 8 carbon atoms in the chain and a substituted or unsubstituted aryl group.

The compounds of the present invention act as both coupler generators and pH modifiers under the following conditions:

(1) Where  $R_1$  and  $R_2$  both are



and  $R_7$  is hydrogen, and

(2) Where either  $R_1$  or  $R_2$  is



and the other group is



Where  $R_3=R_4=H$  and  $R_5$  is an alkyl group having from 1 to 8 carbon atoms in the chain, the compounds are predominantly pH modifiers where the other substituents are as follows:

(a)



2

(b)



and



In all other cases, the compounds act primarily as coupler formers or generators when heated.

10 The temperature at which the present compounds react to function as pH modifiers and/or coupler generators varies, depending on the nature of the substituents, but generally is in the range of from about 75° C. to about 200° C.

15 The essential ingredients of the present compositions are a light-sensitive diazonium salt or mixture of salts and a compound or mixture of compounds selected from the group having the following general formula:



where radicals  $R_1$  through  $R_5$  are groups of the type described above.

25 The essential ingredients are ordinarily combined in a solution of a film-forming resin in a volatile solvent and are applied as a coating onto a suitable substrate. Self-supporting elements may also be produced by coating the composition on a temporary support, drying and then stripping off the film.

While the exact proportions of ingredients are not critical, good results are obtained by combining the ingredients in the following general proportions:

| Ingredient:                             | Percent by weight |
|-----------------------------------------|-------------------|
| Light-sensitive diazonium salt          | 0.2-6.0           |
| See footnote (*)                        | 1.0-20.0          |
| Film-forming natural or synthetic resin | 5.0-40.0          |
| Volatile solvent for resin              | Balance           |



For optimum results, up to a few percent of various other additives, such as a stabilizing acid, cyanoguanidine, zinc chloride, thiourea and other base or coupler generators, may also be added to the composition.

45 A preferred formulation of a satisfactory light-sensitive composition in accordance with this invention is as follows:

| Ingredient:                             | Percent by weight |
|-----------------------------------------|-------------------|
| Light-sensitive diazonium salt          | 0.5-5             |
| See footnote (*)                        | 3-20              |
| Zinc chloride                           | 0-1               |
| Thiourea                                | 0-2               |
| Cyanoguanidine                          | 0-5               |
| Stabilizing acid                        | 0-5               |
| Film-forming natural or synthetic resin | 5-15              |
| Volatile solvent for resin              | Balance           |



65 Among the coupler generator and/or pH modifier compounds suitable for use in the present invention, the following are typical:

1.



## 3



## 4



The coupler generator and/or pH modifier compounds may be prepared according to methods well known in the prior art. For example, the compound represented by formula number 8 above, namely, 3 hydroxyglutaronitrile, may be prepared according to the method disclosed by F. Johnson et al., J. Org. Chem., volume 27, pages 2241-3 (1962). The compound represented by formula number 20, namely,  $\beta$ -hydroxy- $\beta$ -methyl glutaric acid may be prepared according to the method disclosed by Thorne et al., Biochem. Biophys. Acta, volume 59, pages 273-279 (1952) and Wright, Gen. Comp. Endocrinol., volume 1, pages 381-385 (1961).

Under the influence of heat, certain of the present compounds generate a component capable of coupling with a light-sensitive diazonium salt. It is believed that the coupling component is produced by splitting out water, an alcohol or a phenol formed by radical  $R_5O$  and a hydrogen from the carbon to which  $R_4$  is attached. If  $R_4$  is H, loss of water may occur in either direction depending on the nature of  $R_1$  and  $R_2$ . Where  $R_5$  is hydrogen, the by-product is water and where  $R_5$  is an alkyl or aryl group, the by-product is an alcohol or phenol. The splitting out of water or alcohol is attended by the formation of a double bond between the carbon atoms to which groups  $R_3$  and  $R_4$  are attached. This in turn results in the formation of an active methylene group at the carbon adjacent to  $R_1$ . If  $R_4$  is H, the active methylene may be adjacent to either  $R_1$  or  $R_2$ .

It should be understood that the invention does not depend on the accuracy of the stated theory of reaction which is only an attempt to explain the mechanism by which couplers may be generated by heating the present compounds.

In the present compositions, there may be employed conventional light-sensitive diazonium salts which are stable at temperatures of thermal development and which couple with the couplers generated by the present compounds. Such diazonium salts include, for example, p-diazodimethylaniline full zinc chloride, p-diazodiethyl-aniline full zinc chloride, and  $\frac{1}{2}$  zinc chloride, p-diazo-N-ethyl-N-hydroxyethylaniline  $\frac{1}{2}$  zinc chloride, p-diazo-N-methyl-N-hydroxyethylaniline  $\frac{1}{2}$  zinc chloride, p-diazo-diphenylamine sulfate, p-diazo-2,5-diethoxy-benzoyl aniline  $\frac{1}{2}$  zinc chloride, p-diazo-1-morpholino benzene

1/2 zinc chloride, p-diazo-2,5-dimethoxy-1-p-tolyl-mercapto benzene 1/2 zinc chloride, 2,5,4-triethoxy-diphenyl-4-diazonium oxalate, etc.

The following examples will assist towards a full understanding of the present invention. While the examples are not intended to be limiting, they do serve to illustrate certain preferred embodiments of the invention.

## Example 1

10 A 100 ml. solution is prepared which has the following composition:

| Ingredient:                                | Percent by weight |
|--------------------------------------------|-------------------|
| p-Diazodimethylaniline, full zinc chloride | 1                 |
| See footnote (*)                           | 10                |
| Polyvinylbutyral resin                     | 10                |
| Methanol to make up 100 ml. of solution    | Balance           |



The solution is coated on a transparent polyethylene terephthalate substrate and is dried in air for 24 hours. The resulting element is exposed to light through a negative and is then developed by heating with infra-red radiation for 60 seconds at a temperature of 150° C.

## Example 2

30 A 100 ml. solution having the following composition is prepared:

| Ingredient:                                                                     | Percent by weight |
|---------------------------------------------------------------------------------|-------------------|
| p-Diazodiethylaniline, full zinc chloride                                       | 6.0               |
| See footnote (*)                                                                | 20.0              |
| Thiourea                                                                        | 2.0               |
| Citric acid                                                                     | 3.0               |
| Zinc chloride                                                                   | 1.0               |
| Cellulose acetate butyrate                                                      | 15.0              |
| Acetone, methyl ethyl ketone and methanol, ratio 1:1:1 to make 100 ml. solution | Balance           |



The solution is coated, dried, exposed and developed following the procedure of Example 1, except that the 50 temperature of development is 180° C.

## Example 3

55 A 100 ml. solution having the following composition is prepared:

| Ingredient:                                             | Percent by weight |
|---------------------------------------------------------|-------------------|
| p-Diazo-2,5-diethoxy-benzoyl aniline, 1/2 zinc chloride | 3.0               |
| See footnote (*)                                        | 10.0              |
| Tartaric acid                                           | 1.5               |
| Thiourea                                                | 0.5               |
| Zinc chloride                                           | 0.5               |
| Cyanoguanidine                                          | 2.0               |
| Polyvinylbutyral resin                                  | 20.0              |
| Methanol to make 100 ml. of solution                    | Balance           |



The solution is coated, dried, exposed and developed as in Example 1.

## Example 4

A 100 ml. solution having the following composition is prepared:

| Ingredient:                                                                        | Percent by weight |
|------------------------------------------------------------------------------------|-------------------|
| p-Diazo-1-morpholino benzene, 1/2 zinc chloride                                    | 5.0               |
| See footnote (*)                                                                   | 15.0              |
| Thiourea                                                                           | 1.0               |
| Tartaric acid                                                                      | 2.5               |
| Zinc chloride                                                                      | 0.2               |
| Celulose acetate                                                                   | 20.0              |
| Acetone, methyl ethyl ketone and methanol, ratio 1:1:1 to make 100 ml. of solution | Balance           |



The solution is coated, dried, exposed and developed as in Example 1.

## Example 5

A 100 ml. solution having the following composition is prepared:

| Ingredient:                       | Percent by weight |
|-----------------------------------|-------------------|
| p-Diazo-diphenylamine sulfate     | 4.0               |
| See footnote (*)                  | 13.0              |
| Thiourea                          | 1.0               |
| Tartaric acid                     | 3.0               |
| Zinc chloride                     | 0.5               |
| Polyvinylbutyral                  | 15.0              |
| Methanol to make 100 ml. solution | Balance           |



The solution is coated, dried, exposed and developed as in Example 1.

## Example 6

A 100 ml. solution having the following composition is prepared:

| Ingredient:                                 | Percent by weight |
|---------------------------------------------|-------------------|
| p-Diazo-dimethylaniline, full zinc chloride | 3.0               |
| See footnote (*)                            | 10.0              |
| Thiourea                                    | 1.0               |
| Citraconic acid                             | 5.0               |
| Zinc chloride                               | 0.4               |
| Polyvinylbutyral                            | 15.0              |
| Methanol to make 100 ml. solution           | Balance           |



The solution is coated, dried, exposed and developed as in Example 1.

Where the specific compound of the invention is primarily a coupler generator, it will be necessary to add a base generator to the composition. In Examples 3 and 5, for instance, cyanoguanidine and thiourea perform this function.

The compositions of the invention are highly useful in producing all types of light-sensitive, thermo-developable element, such as copy papers, films and the like, which can be developed solely by the application of heat.

It will be understood by those skilled in the art that 70 various modifications may be made in the invention as described and illustrated in the preceding examples without departing from the scope or spirit of the invention as expressed in the following claims.

What is claimed is:

1. A light-sensitive, thermo-developable composition

comprising a light-sensitive diazonium compound and a compound having the following general formula:



5

where  $\text{R}_1$  and  $\text{R}_2$  are radicals selected from the group consisting of



10

and where  $\text{R}_3$ ,  $\text{R}_4$ ,  $\text{R}_5$  and  $\text{R}_6$  are radicals selected from the group consisting of  $-\text{H}$ , an alkyl group having from 1 to 8 carbon atoms in the chain, and an aryl group.

2. A light-sensitive, thermo-developable composition comprising:

from 0.2% to 6.0% by weight of a light-sensitive diazonium compound,

from 1.0% to 20.0% by weight of a compound having 20  
the following general formula:



25

where  $\text{R}_1$  and  $\text{R}_2$  are radicals selected from the group consisting of



and where  $\text{R}_3$ ,  $\text{R}_4$ ,  $\text{R}_5$  and  $\text{R}_6$  are radicals selected from the group consisting of  $-\text{H}$ , an alkyl group having from 1 to 8 carbon atoms in the chain, and an aryl group,

from 5.0% to 40.0% by weight of a film-forming resin, and

the balance a volatile solvent for said resin.

3. A light-sensitive, thermo-developable element comprising a substrate and a coating on at least part of the surface of said substrate, said coating comprising the residue of the composition of claim 2 after evaporation of said volatile solvent.

4. A light-sensitive, thermo-developable element comprising a self-supporting film comprising the residue of the composition of claim 2 after evaporation of said solvent.

#### References Cited

#### UNITED STATES PATENTS

|           |        |                  |       |         |
|-----------|--------|------------------|-------|---------|
| 3,164,468 | 1/1965 | Moskowitz et al. | ----- | 96-49   |
| 3,303,028 | 2/1967 | Aebi et al.      | ----- | 96-49 X |
| 3,307,952 | 3/1967 | Aebi et al.      | ----- | 96-49 X |

NORMAN G. TORCHIN, Primary Examiner.

C. BOWERS, Assistant Examiner.